

# United States Patent Office

3,340,190

Patented Sept. 5, 1967

1

3.340.190

**5,540,190  
RAILWAY DIESEL OIL**

**RAILWAY DIESEL OIL**  
Sigmund S. Deluga, Munster, James W. Harnach, Chesterton, and Randel Q. Little, Jr., Munster, Ind., assignors to Standard Oil Company, Chicago, Ill., a corporation of Indiana

No Drawing. Filed June 1, 1965, Ser. No. 460,549  
11 Claims. (Cl. 252—33.4)

This invention relates to an alkaline lubricating oil and more particularly pertains to lubricating oils of high dispersancy-detergency and high alkalinity for use as crank-case lubricant in heavy duty diesel engines such as railway freight diesel engines.

Heavy duty diesel engines require crankcase lubricant oils which are stabilized against oxidation, are non-corrosive to silver bearings, keep in suspension combustion products which would deposit and/or form as sludge and/or varnish on pistons, cylinder liners and undercrown cavities. The diesel crankcase lubricant should prevent carbon deposition in the top ring piston grooves. The alkalinity life of the crankcase lubricating oil should be long for the purpose of reducing the need to add alkalinity imparting additives before complete change of crankcase lubricant oil or to reduce the frequency of changes of crankcase lubricating oil. In addition the crankcase lubricating oils for heavy duty diesel engines must be so formulated that silver connecting rod bearings and lead surfacing thereon are not attacked either by the additives in the oil formulation or by the dispersed, neutralized or decomposition products thereon during extended use.

The present invention is directed to a unique combination of lubricant oil addition agents dissolved in the required base oils for heavy duty diesel engine crankcase lubrication. The diesel engine crankcase lubricant compositions of this invention when used in field testing in new high speed railway diesel freight engines have demonstrated their ability to maintain a clean engine, provide reserve alkalinity in the used crankcase oil and protect the lead surfaced silver connecting rod bearing even after 77,000 miles of high speed freight service. Most of the parts of one engine replicate of several under test at the same time on the same oil formulation when disassembled showed negligible wear by precise micrometer measurements. That is, after 77,000 miles of high speed services most of the used engine's internal parts were within newly manufactured part tolerance ranges and none showed sufficiently high wear to warrant replacement.

The unique combination of lubricant addition agents according to this invention is a mixture of the exactly neutralized calcium salt of a N,N'-bis(alkyl substituted hydroxybenzyl) alkylene diamine and a bis (alkenylsuccinimide) of polyalkylene polyamine or of a urea condensation derivative of polyalkylene polyamine, N,N'-bis(polyazalkylamino) ureylene. By exactly neutralized calcium salt of N,N'-bis(alkyl substituted hydroxybenzyl) alkylene diamine is meant that calcium salt which contains one gram atom calcium for two molecular equivalents of hydroxyl group, that is one calcium replaces one hydrogen on each of two OH groups. The N,N'-bis (alkyl substituted hydroxybenzyl) alkylene diamines are well known compounds and are generally derived by reacting two moles alkyl substituted phenol, two moles formaldehyde and one mole alkylene diamine such as ethylene diamine, 1,2-diamino-propane, 1,3-diamino-propane, 1,2-diamino-butane, 1,3-diamino-butane, 1,4-diamino-butane, diamino-pentanes, diamino-hexanes, etc. Desirably, these alkylene diamines contain 2 to 10 carbon atoms. Also the alkyl substituent on the benzene ring of the starting phenol and therefore in the N,N'-bis (alkyl substituted hydroxybenzyl) alkylene diamine is de-

sirably of a size (carbon number) to impart oil solubility to the calcium salt. Preferably, the alkyl substituent is alkyl hydrocarbon containing 5 to 70 carbon atoms. Thus the aforementioned exactly neutralized calcium salts can be illustrated by the formula:



wherein "alkylene" is a divalent  $C_2$  to  $C_{10}$  open chain hydrocarbon and R is a  $C_5$  to  $C_{70}$  alkyl hydrocarbon.

15 The bis(alkenylsuccinimide) of polyalkylene polyamines or of urea polyalkylene polyamine condensation derivative are not as easily illustrated by structural formula. In general, they are obtained by reacting about two moles of alkenyl (or alkyl) substituted succinic anhydride with one mole of polyalkylene polyamine. The alkenyl or alkyl substituent on the bis-succinimide also must be of a size (carbon number) to impart oil solubility. For this purpose alkyl or alkenyl groups having at least 30 carbon atoms (about 420 molecular weight) up to 215 carbon atoms (about 3000 molecular weight) are desired. Such  $C_{30}$  to  $C_{215}$  alkyl or alkenyl succinic anhydrides are obtained by reacting in a known manner maleic anhydride with wax hydrocarbons, low molecular weight (M of 420 to 3000) polymers of propylene, isobutylene or copolymers of propylene or isobutylene with a different  $C_2$  to  $C_5$  mono-olefin. The polyalkylene polyamine can be considered a product of the reaction of ammonia and a dihaloalkane, i.e., dichlorethane. Thus the polyalkylene polyamines can be illustrated by the formula:



wherein "alkylene" is a divalent, open chain  $C_2$  to  $C_{10}$  hydrocarbon, R is lower alkyl hydrocarbon (i.e.  $C_1$  to  $C_4$ ) and x is a number of from 2 to 10. Illustrative of these polyalkylene polyamines include diethylene triamine, triethylene tetramine, tetraethylene pentamine, pentaethylene hexamine, heptaethylene octamines (3, 6, 9, 12, 15, 18-hexaethylcane-1,20-diamine), dipropylene triamine, tripropylene tetramine, tetrapropylene pentamine, pentapropylene hexamine and heptapropylene octamine (4, 8, 12, 16, 20, 24-hexazaheptacosane-1,27-diamine) among others.

The urea-polyalkylene polyamine condensation product (polyazalkyl amino) ureylene is obtained according to the method of a contemporary by reacting two moles of polyalkylene polyamine with one mole of urea at temperatures up to about 500° F. accompanied by the evolution of two moles ammonia. From urea and diethylene triamine there is obtained:



which can be named N,N'-bis(5-amino-3-azahethyl)ureylene. For the preparation of these urea-polyalkylene polyamine condensation products the polyalkylene polyamines hereinbefore defined by structural formula are desirable. It will be appreciated that the liberation of ammonia need not come from the terminal NH<sub>2</sub> group of the polyalkylene polyamine but may well come from urea and thus the carboxyl group of urea may be linked to one of the secondary nitrogens in the chain as in:



which can be named 1,3-tetra(2-aminoethyl) urea. From

TABLE I

|                                      | Present Invention Formulation LF | Commercial Formulation A |
|--------------------------------------|----------------------------------|--------------------------|
| Viscosity Index.....                 | 73                               | 67                       |
| Total Base Number <sup>1</sup> ..... | 7.5                              | 6.2                      |
| pH <sup>1</sup> .....                | 11.6                             | 10.4                     |
| Calcium-Weight percent.....          | 0.16                             | 0.21                     |

<sup>1</sup> Method of ASTM-D-664.

the condensation of two moles polyalkylene polyamine (e.g. diethylene triamine) with one mole urea there can be mixtures of (I) and (II) as well as mixtures of (I), (II) and N-(5-amino-3-azaheptyl) N'-(2-amino-ethyl) ureylene. Such mixtures would provide reactive primary amino ( $\text{NH}_2$ ) groups for reaction with the alkyl or alkenyl substituted succinic anhydride:



wherein R is a  $\text{C}_{30}$  to  $\text{C}_{215}$  alkyl or alkenyl hydrocarbon substituent as hereinbefore disclosed to form a disuccinimide.

The preferred combinations of addition agents are the exactly neutralized calcium salt of N,N'-bis( $\text{C}_5$  to  $\text{C}_{70}$  alkyd substituted hydroxybenzyl) ethylene diamine with bis( $\text{C}_{30}$  to  $\text{C}_{215}$  alkenylsuccinimide) of tetraethylene pentamine or with bis( $\text{C}_{30}$  to  $\text{C}_{215}$  alkenyl succinimide) of the N,N'-bis(polyazalkylamino) ureylene derived from two moles tetraethylene pentamine condensed with one mole urea. The most preferred exactly neutralized calcium salts are of N,N'-bis(tert-octylhydroxybenzyl) ethylene diamine, N,N'-bis(nonylhydroxybenzyl) ethylene diamine and N,N'-bis( $\text{C}_{28}$  alkyl hydroxybenzyl) ethylene diamine.

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

mole range of bis-succinimide to calcium gram atom range.

To provide the unique combination of bis-succinimide and calcium salt of bis(alkyl hydroxybenzyl) ethylene diamine there are employed in the range of from 0.001 to 0.01 mole for each 0.025 to 0.05 gram atom of calcium in the calcium salt. More concisely stated, the foregoing ratios are a range of from 0.02 to 0.4 mole bis-succinimide per gram atom of calcium. These ratios of mole ratio range to gram atom range are applicable for additive concentrates, containing 10 to 85% of each additive, to be diluted with lubricant base oil of the 60 to 75 viscosity index range. Usually blends of SAE 30, 40 and/or 50 weight oils are used to prepare railway diesel engine crankcase lubricant oil compositions. The formulation hereinbefore described as "Present Invention Formulation LF" contains the bis-succinimide and calcium salt within said ratios of mole bis-succinimide range to gram atom calcium range. Formulations having said ratios of mole ratio range to gram atom range are prepared from the following specific bis-succinimides and calcium salt of bis(alkyl hydroxybenzyl) ethylene diamines:

*Bis-Succinimide A.*—Solution of 40 weight percent of borated (0.67 weight percent boron) bis-succinimide of tetraethylene pentamine wherein the succinimide groups are derived from 960 molecular weight alkenyl substituted succinic anhydride.

*Bis-Succinimide B.*—Solution of 50 weight percent of bis-succinimide of tetraethylene pentamine wherein the succinimide groups are derived from 960 molecular weight alkenyl substituted succinic anhydride.

*Bis-Succinimide C.*—Solution of 45 weight percent bis-succinimide of amine product of two moles tetraethylene pentamine with one mole urea and the succinimide groups are derived from 960 molecular weight alkenyl substituted succinic anhydride.

*Bis-Succinimide D.*—Solution of 50 weight percent of borated bis-succinimide described for Bis-Succinimide C having a boron to nitrogen weight ratio of about 0.35.

*Calcium amine-coupled phenate.*—A 40 weight percent solution of exactly neutralized calcium salt of N,N'-bis(nonylhydroxybenzyl) ethylene diamine.

Typical concentrations of this invention from the foregoing additives as those resulting from the amounts of each indicated to prepare 100 pounds of concentrate:

|                               | Pounds |
|-------------------------------|--------|
| Bis-Succinimide A             | 17     |
| Calcium amine-coupled phenate | 83     |
| <b>Concentrate A:</b>         |        |
| Bis-Succinimide A             | 41.2   |
| Calcium amine-coupled phenate | 58.8   |
| <b>Concentrate B:</b>         |        |
| Bis-Succinimide B             | 17     |
| Calcium amine-coupled phenate | 83     |
| <b>Concentrate C:</b>         |        |
| Bis-Succinimide B             | 41.2   |
| Calcium amine-coupled phenate | 58.8   |
| <b>Concentrate D:</b>         |        |
| Bis-Succinimide B             | 17     |
| Calcium amine-coupled phenate | 83     |
| <b>Concentrate E:</b>         |        |
| Bis-Succinimide C             | 41.2   |
| Calcium amine-coupled phenate | 58.8   |
| <b>Concentrate F:</b>         |        |
| Bis-Succinimide C             | 17     |
| Calcium amine-coupled phenate | 83     |
| <b>Concentrate G:</b>         |        |
| Bis-Succinimide D             | 41.2   |
| Calcium amine-coupled phenate | 58.8   |
| <b>Concentrate H:</b>         |        |
| Bis-Succinimide D             | 17     |
| Calcium amine-coupled phenate | 83     |

The foregoing concentrates contain the mole of bis-succinimide and gram atom (g.a.) of calcium as shown in Table III.

TABLE III  
MOLE BIS-SUCCINIMIDE AND GRAM ATOM CALCIUM  
PER 100 GRAMS CONCENTRATE

| Concentrate | Bis-Succinimide-Mole | Calcium-Gram Atom | Mole per g.a. Ca |
|-------------|----------------------|-------------------|------------------|
| A           | 0.0028               | 0.059             | 0.047            |
| B           | 0.0068               | 0.042             | 0.16             |
| C           | 0.0034               | 0.059             | 0.058            |
| D           | 0.0081               | 0.042             | 0.198            |
| E           | 0.0026               | 0.059             | 0.044            |
| F           | 0.0068               | 0.042             | 0.15             |
| G           | 0.003                | 0.059             | 0.051            |
| H           | 0.0074               | 0.042             | 0.176            |

The foregoing concentrates are diluted with a base oil blend having a viscosity index of 73. In the following formulations said blend is referred to as "73 VI Base Oil."

|                |        |
|----------------|--------|
| Formulation 1: | Pounds |
| Concentrate A  | 100    |
| 73 VI Base Oil | 1450   |
| Formulation 2: |        |
| Concentrate B  | 100    |
| 73 VI Base Oil | 900    |
| Formulation 3: |        |
| Concentrate C  | 100    |
| 67 VI Base Oil | 1450   |
| Formulation 4: |        |
| Concentrate D  | 100    |
| 68 VI Base Oil | 900    |
| Formulation 5: |        |
| Concentrate E  | 100    |
| 71 VI Base Oil | 1450   |
| Formulation 6: |        |
| Concentrate F  | 100    |
| 73 VI Base Oil | 900    |
| Formulation 7: |        |
| Concentrate G  | 100    |
| 73 VI Base Oil | 1450   |
| Formulation 8: |        |
| Concentrate H  | 100    |
| 73 VI Base Oil | 900    |

In the foregoing Formulations 1, 3, 5 and 7 have about 1.0 weight percent of the respective bis-succinimides and Formulations 2, 4, 6 and 8 have about 4.0 weight percent bis-succinimides.

The combination of addition agents of this invention give outstanding performance in diesel engine crankcase lubricating oil compositions in actual service conducted under severe conditions. To illustrate this, the results of the use of a typical formulation, e.g., Formulation 1 is herein-after set forth. The test employed is known as the 300 hour EMD 2-567 Engine Performance Test (EMD is Electro-Motive Division of General Motors). In this test the diesel engine crankcase of a clean engine having new moving parts and bearings is filled with the lubricating oil composition. The engine is started and operated for 9 hours and 20 minutes under break in conditions at the end of which an engine speed of 835 r.p.m. and load of 210 horsepower is achieved. Then the engine is operated at 835 r.p.m. with a steady 210 horsepower load, engine cooling water at 195° F. and oil sump temperature of 240° F. for 300 hours. During the test samples of the used oil are taken at 100, 200 and 300 hours of operation. These samples are subject to evaluation for SSU (Saybolt Seconds Universal) at 100° F. and 210° F. to determine percent viscosity change, the weight percent pentane and benzene insolubles content, the total acid number, the total base number and pH of the used oil composition. At the end of the 300 hour test under load, the engine is disassembled and its parts are inspected for piston groove filling, deposits on land above top ring, deposit under piston crown, piston skirt discoloration (evaluated on a 0 to 800 scale where 0 is clean and 800 is black), oil filter screen deposits and filter condition, bearings performance, and general corrosion as well as corrosion of bronze thrust washer

and copper-lead camshaft bearings. The results of this test are as follows:

## EMD 2-567 ENGINE PERFORMANCE

## Engine deposits:

|                                      |        |
|--------------------------------------|--------|
| Piston ring groove filling, percent: |        |
| Top ring                             | 73     |
| No. 2 ring                           | 90     |
| No. 3 ring                           | 36     |
| Land above top ring, percent filled  | 13     |
| Piston discoloration No.:            | 740    |
| (0=clean, 800=black)                 | <0.002 |
| Undercrown deposit thickness, in.    | None   |
| Oil screen deposits, percent         | Good   |
| Oil filter condition                 |        |

## Bearing performance:

|                                                                               |      |
|-------------------------------------------------------------------------------|------|
| Silver bearing type                                                           |      |
| Right bearing weight loss 0-300 hours, gram                                   | 0.24 |
| Weight loss leaded insert (lead overlay intact)                               | 0.57 |
| Metallurgical inspection of unleaded insert at 300 hours—no silver corrosion. |      |
| Bronze thrust washer average weight loss, gram                                | 0.32 |
| Metallurgical inspection—no sulfidic attack.                                  | 25   |
| Copper-lead camshaft bearings average weight loss 0-300 hours, gram           | 0.02 |
| Metallurgical inspection—no corrosion.                                        |      |

EMD 2-567 ENGINE PERFORMANCE (CONTINUED)  
[Used Oil Inspections]

|                                         | Viscosity, SSU      |                   |      |
|-----------------------------------------|---------------------|-------------------|------|
|                                         | 100° F.             | 210° F.           |      |
| Hours:                                  |                     |                   |      |
| 0                                       | 1,038               | 79.7              |      |
| 100                                     | 1,116               | 82.7              |      |
| 200                                     | 1,141               | 84.0              |      |
| 300                                     | 1,166               | 84.9              |      |
| Percent Viscosity Increase at 300 Hours | 12                  | 7                 |      |
|                                         | Insolubles, Percent |                   |      |
|                                         | Pentane             | Benzene           |      |
| Hours:                                  |                     |                   |      |
| 100                                     | 0.10                | 0.10              |      |
| 200                                     | 0.09                | 0.05              |      |
| 300                                     | 0.15                | 0.07              |      |
|                                         | Acidity             |                   |      |
|                                         | Total Acid Number   | Total Base Number | pH   |
| Hours:                                  |                     |                   |      |
| 0                                       | 0                   | 7.80              | 11.1 |
| 100                                     | 0.79                | 3.01              | 8.6  |
| 200                                     | 0.95                | 2.16              | 8.4  |
| 300                                     | 0.89                | 1.68              | 8.8  |

A lubricant oil composition of this invention was field tested as crankcase lubricating oil in eight new diesel electric freight locomotives each equipped with one Electro-Motive Division of General Motors 16 cylinder type 567-D3A turbocharged diesel engine. After delivery to Railroad Company the initial fill crankcase oil was drained and filled with lubricant oil Formulation 1. These freight locomotives were placed in transcontinental high speed service. At the end of about five months service the mileage of use of the eight locomotives varied from 68,000 to 80,000 miles. At this time one locomotive, hereinafter referred to as Locomotive 85, was available in the locomotive shops of Railroad Company for a field test interim inspection. Locomotive 85 had accumulated about 77,000 miles of service with about 80% of working

time in eighth throttle notch, full power setting of throttle and had experienced no oil drain and refills.

Inspections were made of top deck, cover and air box of Locomotive 85. Negligible deposits were found on the top deck and cover and these deposits were easily removed by wiping which left clean bare metal. Deposits in air boxes were only thin where deposits were found tapering to clean metal areas.

The condition of pistons and rings were evaluated by inspection through engine ports. All of the piston rings showed initial machinery marks which is indicative of low wear. All the rings were bright, metallic in appearance indicative of satisfactory ring function.

Power assemblies in positions Numbers 6 and 14 were removed for deposit and wear measurements. The excellent results are seen from the following summarized evaluations:

ENGINE DEPOSIT RATINGS<sup>a</sup>

|    |         |                                                       |       |
|----|---------|-------------------------------------------------------|-------|
| 20 | Piston: | Ring + groove deposits, percent filled <sup>b</sup> : |       |
|    |         | Number 1                                              | 85    |
|    |         | Number 2                                              | 60    |
|    |         | Number 3                                              | 40    |
|    |         | Number 4                                              | 10    |
|    |         | Number 5                                              | 0     |
|    |         | Number 6                                              | 0     |
|    |         | Skirt deposits <sup>c</sup>                           | 190   |
|    |         | Undercrown deposits, average thickness, inches        | 0.004 |

30 Liner port restriction—None.

Valve deposits—Negligible.

Top deck—Wipeable oil, clean.

Top deck cover—Wipeable oil, clean.

35 <sup>a</sup> Average of two power assemblies.

<sup>b</sup> 100% filled=0.054".

<sup>c</sup> 0=no deposit, 400=100% covered brown deposit, 800=100% covered black deposit.

ENGINE WEAR MEASUREMENTS<sup>1</sup>  
[Inch]

|    |                         | Typical New Part |       |
|----|-------------------------|------------------|-------|
|    |                         |                  |       |
| 45 | Ring Gaps: <sup>2</sup> |                  |       |
|    | No. 1                   | 0.045            | 0.04  |
|    | Avg. 1, 2, 3, 4         | 0.042            | 0.04  |
| 45 | Ring-Groove Clearance:  |                  |       |
|    | No. 1                   | 0.009            | 0.007 |
|    | Avg. 2, 3, 4            | 0.010            | 0.010 |
| 50 | Piston Groove Width:    |                  |       |
|    | No. 1                   | 0.198            | 0.196 |
|    | Avg. 1, 2, 3, 4         | 0.196            | 0.196 |
| 50 | Piston Skirt Diameter   | 8.486            | 8.489 |
|    | Cylinder Liner Diameter | 8.502            | 8.501 |
|    | Thrust Washer           | 0.186            | 0.186 |
|    | Silver Bearing          | (3)              | (3)   |

1 Average of two power assemblies.

2 Machine marks 100% visible.

3 Lead overlay 90% intact. No corrosion or wiping of exposed silver.

55 The data show that the engine was exceptionally clean. There were moderate deposits in compression ring grooves; however, the oil control rings and grooves were completely clean. Piston skirts were clean with skirt deposits covering less than 20% of the total area. Inlet port and valve deposits were negligible.

60 The silver bearings were in excellent condition. The lead flashing still covered about 90% of the total area, and where free silver was exposed, there was no evidence of corrosion or wiping. The rod bearings and slipper bearing surface showed no evidence of wear. The thrust washer also looked satisfactory and measured within new tolerance limits. The pistons, rings and liners showed little or no wear. The addition of about 0.2 to 1.0 desirably 0.3 to 0.8 and preferably 0.4 to 0.8, weight percent oil-soluble calcium salt of alkyl (C<sub>12</sub> to C<sub>30</sub>) benzene sulfonic acid to Formulations 1 through 4 may favorably effect reduction of ring carbon deposit.

65 As indicated in the description of bis-succinimides A and D, the bis-succinimide product of reacting the alkyl

or alkenyl substituted succinic anhydride with polyalkylene polyamine or preferably the polyalkylene polyamine-urea condensation product can be modified by boration. This boration is accomplished by the use of boron acid in an amount to provide 0.1 to 1.0 weight percent boron.

What is claimed is:

1. A lubricant composition comprising a lubricating mineral oil having dissolved therein as its essential additive ingredients a combination consisting of the exactly neutralized calcium salt of a N,N'-bis(alkyl substituted hydroxybenzyl) alkylene diamine and a bis(alkenyl substituted succinimide) of a (polyazalkyl amino)-ureylene that is a condensation product of two moles of polyalkylene polyamine with one mole urea, wherein said alkyl substituted hydroxybenzyl the alkyl substituent is alkyl hydrocarbon of from 5 to 70 carbon atoms, wherein said alkylene diamine the alkylene group is a divalent open chain hydrocarbon of from 2 to 10 carbon atoms, wherein said alkenyl substituent of said succinimide has from 30 to 215 carbon atoms and wherein said polyalkylene polyamine has the formula



wherein "alkylene" is a divalent open chain hydrocarbon of from 2 to 10 carbon atoms, R is selected from the class consisting of hydrogen and lower alkyl hydrocarbon of 1 to 4 carbon atoms and x is a number of from 2 to 10; wherein said combination there is present in the range of from 0.02 to 0.4 mole of said bis(alkenyl substituted succinimide) per gram atom of calcium of said exactly neutralized calcium salt; and wherein said lubricant composition there is present from 0.5 to 10 weight percent of said bis(alkenyl substituted succinimide).

2. The composition of claim 1 wherein there is present said bis(alkenyl substituted succinimide) in the range of from 1.0 to 5.0 weight percent.

3. The composition of claim 1 wherein the lubricating mineral oil has a viscosity index of 60 to 75 and there is present from 0.5 up to 10 weight percent of said bis(alkenyl substituted succinimide).

4. The composition of claim 1 wherein said bis(alkenyl substituted succinimide) is as bis(polybutenyl substituted succinimide) whose polybutenyl succinic anhydride moiety has a molecular weight of about 960 and is the succinimide of the amine derived by reacting tetraethylene pentamine with urea in the ratio of two moles of said pentamine per mole urea accompanied by the evolution of two moles ammonia for each mole urea.

5. The composition of claim 4 wherein said bis-succinimide is modified with 0.5 to 0.7 weight percent of boron.

6. The composition of claim 1 wherein said exactly neutralized calcium salt is the exactly neutralized calcium salt of N,N'-bis(nonyl hydroxybenzyl) ethylene diamine.

7. The composition of claim 1 wherein said bis(alkenyl substituted succinimide) is a bis(polybutenyl substituted succinimide) whose polybutenyl succinic anhydride moiety has a molecular weight of about 960 and is the succinimide of the amine derived by reacting tetraethylene pentamine with urea in the ratio of two moles of said

pentamine per mole urea accompanied by the evolution of two moles ammonia for each mole urea, and said exactly neutralized calcium salt is the exactly neutralized calcium salt of N,N'-bis(nonyl hydroxybenzyl) ethylene diamine.

8. A concentrate comprising 10 to 85% by weight of the exactly neutralized calcium salt of a N,N'-bis(alkyl substituted hydroxybenzyl) alkylene diamine and of a bis(alkenyl substituted succinimide) of a (polyazalkyl amino)-ureylene that is a condensation product of two moles of polyalkylene polyamine with one mole urea, wherein said alkyl substituted hydroxybenzyl the alkyl substituent is alkyl hydrocarbon of from 5 to 70 carbon atoms, wherein said alkylene diamine the alkylene group is a divalent open chain hydrocarbon of from 2 to 10 carbon atoms, wherein said alkenyl substituent of said succinimide has from 30 to 215 carbon atoms and wherein said polyalkylene polyamine has the formula



wherein "alkylene" is a divalent open chain hydrocarbon of from 2 to 10 carbon atoms, R is selected from the class consisting of hydrogen and lower alkyl hydrocarbon of 1 to 4 carbon atoms and x is a number of from 2 to 10; and said bis-succinimide is present in an amount to provide 0.02 to 0.4 mole per gram atom of said exactly neutralized calcium salt.

9. The concentrate of claim 8 also containing a calcium salt of a C<sub>12</sub> to C<sub>30</sub> alkyl substituted benzene sulfonic acid in an amount when the concentrate is diluted with a SAE 30 to SAE 50 base oil said calcium sulfonate is present in a concentration of from 0.2 to 1.0% by weight.

10. A lubricant composition comprising a major amount of a mineral lubricating oil of SAE 30 to SAE 50, 0.5 to 10% by weight of a bis(polybutenyl substituted succinimide) of a (polyazalkyl amino)-ureylene prepared from one mole urea and two moles of tetraethylene pentamine whose polybutenyl substituted succinic acid moiety has a molecular weight of about 960 and an amount of exactly neutralized calcium salt of N,N'-bis(nonyl hydroxybenzyl) ethylene diamine to provide for each gram atom of calcium from 0.02 to 0.4 mole of said bis-succinimide.

11. The composition of claim 10 wherein there is also present 0.02 to 1.0 weight percent of the calcium salt of a C<sub>12</sub> to C<sub>30</sub> alkyl substituted benzene sulfonic acid.

#### References Cited

#### UNITED STATES PATENTS

|           |         |               |       |            |
|-----------|---------|---------------|-------|------------|
| 2,353,491 | 7/1944  | Oberright     | ----- | 252—42.7   |
| 3,036,003 | 5/1962  | Verdol        | ----- | 252—33.4   |
| 3,087,936 | 4/1963  | Le Suer       | ----- | 252—32.7 X |
| 3,154,560 | 10/1964 | Osuch         | ----- | 252—51.5 X |
| 3,219,666 | 11/1965 | Norman et al. | ----- | 252—51.5 X |
| 3,272,743 | 9/1966  | Norman et al. | ----- | 252—32.5   |

#### FOREIGN PATENTS

|         |        |                |
|---------|--------|----------------|
| 998,869 | 7/1965 | Great Britain. |
|---------|--------|----------------|

DANIEL E. WYMAN, Primary Examiner.

P. P. GARVIN, Assistant Examiner.